

# UNITED STATES PATENT OFFICE.

PERCY A. E. ARMSTRONG, OF LOUDONVILLE, NEW YORK.

## ELECTRICAL HEATING ELEMENT.

1,416,436.

Specification of Letters Patent. Patented May 16, 1922.

No Drawing. Application filed May 1, 1919, Serial No. 293,927. Renewed October 1, 1921. Serial No. 504,676.

*To all whom it may concern:*

Be it known that I, PERCY A. E. ARMSTRONG, a subject of the King of Great Britain, and a resident of Loudonville, county 5 of Albany, State of New York, have invented certain new and useful Improvements in Electrical Heating Elements, of which the following is a specification.

My invention relates to electrical heating 10 elements.

I have discovered that alloys of iron and chromium have high specific resistance and are practically non-oxidizing and non-corrosive up to about 1300° F. Higher temperatures can be used, but the properties of these 15 alloys are not so desirable for electrical heating units at temperatures substantially higher than 1300° F., say, from about 1600°-1800° F., particularly when run continuously for many hours at a time. 20

The quantity of chromium used depends on the uses to which the heating element is put.

For electrical heating elements to be run at 25 comparatively low temperatures, the proportion of chromium may be low, say from about 4% upwards. For higher temperatures, the proportion of chromium should be greater, and from about 12% of chromium and upwards 30 for "red heat" elements gives good results. At present relative costs, about 30% to 40% chromium content is about the limit for economical production but, if desired, more chromium can be used, practically up 35 to 95% or even 100% chromium, though it is to be understood that I do not claim the use of chromium *per se* as an electrical heating element, but only chromium when alloyed with iron and carbon. Also the higher 40 chromium material is more difficult to work mechanically.

When iron-chromium alloys are worked in heated state, as by forging, for example, there is a considerable production of oxides, 45 scale and the like. When electrically heated, however, without working, these materials are substantially free from oxidation and corrosion and, having substantially high specific resistance, are well adapted for use 50 as electrical heating elements. The fact that they oxidize and scale when worked at high temperatures, together with the known susceptibility of iron itself to scaling and oxidizing at high temperatures, has apparently 55 been responsible for failure heretofore of

investigators in this field to discover the adaptability of these alloys for use as electrical heating elements.

The carbon content preferably does not exceed a maximum of about 1% which is 60 permissible in alloys containing about 12% of chromium or over, though lower carbon, say from about .10%-.60% is better in such material. Silicon up to about .45% in the material having 12% or more of chromium 65 and proportionately lower silicon in lower chromium material down to about .20% or less in 4% chromium material does not materially affect the alloy when made use of as a heating element. 70

Other metals, such as nickel, molybdenum, tungsten, etc., may be present in small quantities up to about 2-4% without marked effect on the qualities of the heating element. Small quantities of various impurities such 75 as phosphorus, copper, tin and the like, may, of course, be present, but are preferably reduced to the minimum conformable with economical production of the material.

It will be seen that my new heating element containing as it does, a large proportion of iron, is of low cost as compared with the expensive alloys heretofore used for this purpose. I find, for example, that a heating element such as described and containing only about 14% of chromium and the principal part of the remainder iron has substantially the same qualities and usefulness as a heating element containing several times as much chromium, and also containing a large quantity of nickel, which is likewise highly expensive, as compared with iron. 85 90

I claim:

1. An electrical heating element containing over 4% of chromium, carbon over .1%, and the principal part of the remainder iron. 95
2. An electrical heating element containing 12% or more of chromium, .1% or more of carbon, and the principal part of the remainder iron. 100
3. An electrical heating element containing about 14% of chromium, about .1% to .6% of carbon and the principal part of the remainder iron. 105

In testimony that I claim the foregoing I hereto set my hand, this 29th day of April, 1919.

PERCY A. E. ARMSTRONG.